

1

3,108,043

**SPERMICIDAL SHEET-LIKE MATERIAL**

Nathan Millman, Somerville, and Roger Edwin Homm, Neshanic, N.J., assignors to Ortho Pharmaceutical Corporation, a corporation of New Jersey

No Drawing. Filed May 9, 1960, Ser. No. 27,507

7 Claims. (Cl. 167—58)

The present invention relates to a novel and improved 10 spermicidal manufacture for treatment of the vaginal cavity to be acted on by the body fluids and provide a convenient and effective spermicidal composition.

Objects and advantages of the invention will be set forth in part hereinafter and in part will be obvious herefrom, or may be learned by practice with the invention, the same being realized and attained by means of the steps, processes and compositions pointed out in the appended claims.

The invention consists in the novel steps, processes, compositions and improvements herein shown and described.

The present invention has for its object the provision of a novel and improved composition and article of manufacture for the convenient treatment of the vaginal cavity to provide it with a readily available and regulated amount of a spermicidal material. A further object is the provision of an economical and conveniently usable material which is adapted to dissolve at a controlled rate in the normal fluids available in the vaginal cavity thereby supplying the cavity with a regulated amount of spermicide. Still another object is the provision of a solid material which is substantially dry, may be inexpensively packaged, which requires no apparatus for its proper and effective use, and which is without deleterious effect on the tissues with which it may remain in contact.

According to the present invention the spermicidal manufacture comprises a non-deleterious, bland mass, which is soluble in the body fluids available in the vaginal cavity at a controlled rate of solution and which incorporates within it an effective amount of a spermicide, together, if desired, with a suitable humectant or plasticizing agent for the mass to maintain the mass in a more pliable, less rigid condition. The spermicidal manufacture is formed into sheets or foams in such a manner that it has an extremely large surface area with respect to its mass, thereby increasing not only the rate at which it may be dissolved on contact with the body fluids, but also rendering the mass more pliable and less likely to cause damage to the tissues with which it comes in contact.

The water soluble solid material which forms the vehicle for the spermicide and which forms the mass is a bland, non-deleterious, solid, film-forming material, which is readily soluble in water and the body fluids with which it comes in contact within the vaginal cavity. Among the soluble materials which have been found suitable are the various viscosity grades of sodium carboxymethylcellulose and methylcellulose. The sodium carboxymethylcellulose and methylcellulose used are of grade having a viscosity of from 25 to 10,000 centipoises per second in a 2% aqueous solution at 25° C., and preferably such that a 2% by weight solution in water at 25° C. has a viscosity of from 25 to 50 centipoises per second, although other grades with similarly measured viscosities of from 50 to 10,000 centipoises per second are usable in certain formulations. Alternatively, they may be employed as vehicles, if desired, other water soluble non-putrefying, bland, film-forming, solid materials such as alginates, cellulose acetate, sorbate, and polyvinyl alcohol (4-6 c.p.s.).

The water soluble vehicle is dissolved and mixed with

2

a suitable water soluble spermicide, such as a non-ionic detergent.

The weight ratio of spermicide to vehicle may be as great as 1:1. It has been found that many spermicides are not compatible with the vehicle when present in larger quantities. The minimum amount of spermicide present should not be less than 5 milligrams per application. Thus, if the total weight of a single film or foam designed for one application were 720 milligrams, the minimum amount of spermicide present should not be less than 5 milligrams. Another way of expressing this relationship is that the weight ratio of spermicide to total solids is not less than about 1:145.

Any water soluble, non-deleterious spermicide may be used, but the non-ionic detergent spermicides are preferred and are selected from the group consisting of diisobutylphenoxypropoxyethoxyethanol described in United States Patent No. 2,752,284, alkylated aryl polyether alcohols, sodium alkylaryl polyether sulfates, and nonylphenoxypropoxyethoxyethanol.

It is preferred that a suitable plasticizer or humectant be added to the water soluble vehicle to render the unmoistened sheet material more pliable and less likely to cause damage to any body tissue with which it may come in contact. Suitable materials for this purpose are glycerol, sorbitol, polyethylene glycols of high molecular weight and other bland, non-deleterious, hygroscopic liquids which are compatible with the film-forming material. The weight ratio of glycerol to vehicle may be as much as 1:1.3 or as little as 1:3. Larger amounts of glycerol are not readily compatible with the vehicle and smaller amounts of glycerol do not produce the desired flexibility.

The solubility of the composition and articles of the present invention in water and body fluids may be controlled by the presence in the vehicle of urea. The amount of urea should be such that a 3-inch square film of the vehicle will dissolve in water at 37° C. in less than 100 seconds. The weight ratio of urea to vehicle may be as much as 1:3 or as little as 1:4. If the ratio of urea to vehicle is greater than 1:3, discontinuity may appear in the cast film. If the ratio of urea to vehicle is less than 1:4, the rate of solubility may be too slow.

The spermicidal manufacture may be formed as a film-like sheet, or as a sheet of foam, but in any event has an extremely large ratio of surface to volume so that it has a large surface which may be acted upon by the solvent fluids to speed the process of dissolution upon contact with the vaginal fluids.

In use, a suitable quantity of the sheet-like material comprising the water soluble sheet containing the spermicide is compacted, either by rolling or by crumpling, and is introduced into the vaginal cavity and immediately begins to dissolve and thus provides a viscous, retained gel, having effective spermicidal activity, on the vaginal walls.

In general, the material of the present invention comprises a sheet of the water soluble vehicle, either sodium carboxymethylcellulose or methylcellulose. The sodium carboxymethylcellulose or methylcellulose which forms the vehicle is preferably dissolved in water to form a solution containing from 0.5% to 12.0% of vehicle solids, together with urea, a humectant such as glycerol, ethylene glycol or sorbitol and a spermicide in the proportions described above.

Where the sheet material is to be in the form of a film, the solution may be poured or otherwise fed onto a heated surface to the correct thickness to give the desired film thickness after drying, and the water is then evaporated by gently heating of the support and the solution carried thereby. The solution is deposited in such

thickness that after drying, the dried film will have a thickness of from 0.001 inch to 0.0075 inch and which will dissolve more rapidly than films having a greater thickness.

Sheets of dried foamed material absorb moisture more readily, films are more supple and in many cases may be preferred for this reason. Such foams or foamed sheet may be produced by violently beating air into the prepared solution comprising all of its ingredients, after which the foamed material is poured out onto a hot surface from which it may eventually be separated, after which the foam or sheet is dried. The heated surface is preferably heated just slightly below the boiling point of water so that the foam is destroyed immediately adjacent the supporting surface to give added strength to the sheet as a whole. Thereafter, the sheet or film is dried in any conventional drying oven or chamber. In the case of a foam, the preferable form is a sheet, relatively thin (from 0.005 inch to 0.240 inch thickness) which has one of its faces substantially continuous and not interrupted by any foam-like or cellular formation, while its other surface exhibits the normal appearance of a dried foam.

Foaming agents may of course be used to assist in the manufacture of a foamed spermicide. It will be appreciated that many active spermicides are surface active

agents and will function as foaming agents in the solution described.

Conveniently, either the non-foamed or the foamed sheet-like material may be cast and dried upon a large heated cylinder having a polished surface, as is customary in connection with the casting of continuous webs of film

A spermicide manufacture of the present invention is made from a water solution comprising:

|    |                                    |             |      |
|----|------------------------------------|-------------|------|
| 10 | Sodium carboxymethylcellulose      | milligrams  | 300  |
|    | Nonylphenoxy polyethoxyethanol     | do          | 100  |
|    | Glycerine (or polyethylene glycol) | do          | 220  |
|    | Urea                               | do          | 100  |
|    | Water                              | milliliters | 46.2 |

15 This solution is dried to form a film 3-inches square and about 0.005 inch in thickness. The ratio of the spermicide present in the dried film to sodium carboxymethylcellulose is 1:3. The ratio of urea to carboxymethylcellulose is also 1:3. The ratio of glycerol (or 20 polyethylene glycol) to sodium carboxymethylcellulose is about 1:1.36.

25 Referring now in detail to various working examples of the manner in which the spermicidal materials of the present invention may be prepared, and the process by which they may be prepared, the following specific ex-

| Film No.                                     | 1     | 2     | 3     | 4     | 5     | 6     | 7    | 8     | 9     | 10    | 11   | 12  |
|----------------------------------------------|-------|-------|-------|-------|-------|-------|------|-------|-------|-------|------|-----|
| Sodium carboxymethylcellulose, 50 centipoise | 0.5   | 1.0   | 2.0   | 5.0   | 12.0  | 12.0  | 12.0 | 12.0  | 0.5   | 0.5   | 1.0  | 2.0 |
| Methylcellulose, 4,000 centipoise            |       |       |       |       |       |       |      |       |       |       |      |     |
| Glycerol                                     | 0.25  | 5.0   | 1.0   | 2.0   | 4.0   | 4.0   | 4.0  | 4.0   | 0.4   | 0.3   | 0.5  | 1.0 |
| Urea                                         | 0.15  | 0.25  | 0.5   | 1.5   | 4.0   | 4.0   | 4.0  | 4.0   | 0.4   | 0.3   | 0.5  | 1.0 |
| Diisobutylphenoxypolyethoxy ethanol          | 0.5   | 1.0   | 2.0   | 5.0   | 0.5   | 1.0   | 2.0  | 5.0   | 0.5   | 0.15  | 0.25 | 0.5 |
| Nonylphenoxypolyethoxy ethanol               |       |       |       |       |       |       |      |       |       |       |      |     |
| Sodium alkaryl polyether sulfate             |       |       |       |       |       |       |      |       |       |       |      |     |
| Alkylated aryl polyether alcohols            |       |       |       |       |       |       |      |       |       |       |      |     |
| Water                                        | 100   | 100   | 100   | 100   | 100   | 100   | 100  | 100   | 100   | 100   | 100  | 100 |
| Glycerol:vehicle                             | 1:2   | 1:2   | 1:2   | 1:2.5 | 1:3   | 1:3   | 1:3  | 1:3   | 1:1.7 | 1:1.7 | 1:2  | 1:2 |
| Urea:vehicle                                 | 1:3.3 | 1:4   | 1:4   | 1:3.3 | 1:3   | 1:3   | 1:3  | 1:3   | 1:3.3 | 1:3.3 | 1:4  | 1:4 |
| Spermicide:vehicle                           | 1:10  | 1:1   | 1:1   | 1:1   | 1:24  | 1:12  | 1:6  | 1:2.5 | 1:1   | 1:1   | 1:1  | 1:1 |
| Thickness of dried film in mils              | 1.0   | 1.5   | 2.0   | 5.0   | 7.5   | 7.5   | 7.5  | 7.5   | 1.0   | 1.0   | 1.5  | 2.0 |
| Film No.                                     | 13    | 14    | 15    | 16    | 17    | 18    | 19   | 20    | 21    | 22    | 23   | 24  |
| Sodium carboxymethylcellulose, 50 centipoise | 5.0   | 12.0  | 5.0   | 5.0   | 12.0  | 12.0  | 12.0 | 12.0  |       |       |      |     |
| Methylcellulose, 4,000 centipoise            |       |       |       |       |       |       |      |       |       |       |      |     |
| Glycerol                                     | 2.0   | 3.0   | 2.0   | 3.0   | 4.0   | 4.0   | 4.0  | 4.0   | 2.0   | 1.0   | 2.0  | 3.0 |
| Urea                                         | 1.66  | 4.0   | 1.6   | 1.67  | 3.0   | 3.0   | 3.0  | 3.0   | 0.33  | 0.66  | 1.0  |     |
| Diisobutylphenoxypolyethoxy ethanol          | 5.0   | 1.0   | 5.0   | 5.0   | 0.5   | 1.0   | 2.0  | 5.0   | 0.33  | 0.66  | 1.0  | 1.0 |
| Nonylphenoxypolyethoxy ethanol               |       |       |       |       |       |       |      |       |       |       |      |     |
| Sodium alkaryl polyether sulfate             |       |       |       |       |       |       |      |       |       |       |      |     |
| Alkylated aryl polyether alcohols            |       |       |       |       |       |       |      |       |       |       |      |     |
| Water                                        | 100   | 100   | 100   | 100   | 100   | 100   | 100  | 100   | 100   | 100   | 100  | 100 |
| Glycerol:vehicle                             | 1:2.5 | 1:3   | 1:2.5 | 1:1.7 | 1:3   | 1:3   | 1:3  | 1:3   | 1:2   | 1:3   | 1:3  | 1:3 |
| Urea:vehicle                                 | 1:3   | 1:3   | 1:3.1 | 1:3   | 1:4   | 1:4   | 1:4  | 1:4   | 1:4   | 1:3   | 1:3  | 1:3 |
| Spermicide:vehicle                           | 1:1   | 1:1   | 1:1   | 1:1   | 1:24  | 1:12  | 1:6  | 1:2.4 | 1:1   | 1:1   | 1:2  | 1:3 |
| Thickness of dried film in mils              | 5.0   | 7.5   | 5.0   | 5.0   | 7.5   | 7.5   | 7.5  | 7.5   | 2.0   |       |      |     |
| Film No.                                     | 25    | 26    | 27    | 28    | 29    | 30    | 31   | 32    | 33    | 34    | 35   | 36  |
| Sodium carboxymethylcellulose, 50 centipoise |       |       | 10.0  | 10.0  | 10.0  | 2.0   | 2.0  | 2.0   |       | 2.0   | 2.0  |     |
| Methylcellulose, 4,000 centipoise            | 4.0   | 5.0   |       |       |       |       |      |       |       |       |      |     |
| Glycerol                                     | 2.0   | 2.0   | 3.3   | 6.0   | 8.0   | 1.0   | 1.0  | 1.0   | 2.0   |       |      | 2.0 |
| Urea                                         | 1.0   | 1.67  | 3.0   | 2.5   | 3.3   | 0.5   | 0.5  | 0.5   | 1.0   | 1.0   | 1.0  | 1.0 |
| Diisobutylphenoxypolyethoxy ethanol          | 1.0   | 1.0   | 5.0   | 2.0   | 1.0   |       |      | 2.0   |       | 2.0   |      | 0.5 |
| Nonylphenoxypolyethoxy ethanol               |       |       |       |       |       |       |      |       |       |       |      |     |
| Sodium alkaryl polyether sulfate             |       |       |       |       |       |       |      |       |       |       |      |     |
| Alkylated aryl polyether alcohols            |       |       |       |       |       |       |      |       |       |       |      |     |
| Water                                        | 100   | 100   | 100   | 100   | 100   | 100   | 100  | 100   | 100   | 100   | 100  | 100 |
| Glycerol:vehicle                             | 1:2   | 1:2.5 | 1:3   | 1:1.5 | 1:1.2 | 1:2   | 1:2  | 1:2   | 1:2   | 1:2   | 1:2  | 1:2 |
| Urea:vehicle                                 | 1:4   | 1:3   | 1:3.3 | 1:4   | 1:3   | 1:4   | 1:4  | 1:4   | 1:4   | 1:4   | 1:4  | 1:4 |
| Spermicide:vehicle                           | 1:4   | 1:5   | 1:2   | 1:5   | 1:10  | 1:1   | 1:1  | 1:1   | 1:1   | 1:1   | 1:1  | 1:1 |
| Thickness of dried film in mils              |       |       |       | 5.0   | 5.0   | 2.0   | 2.0  | 2.0   | 2.0   | 2.0   | 2.0  | 2.0 |
| Film No.                                     | 37    | 38    | 39    | 40    | 41    | 42    | 43   | 44    | 45    | 46    | 47   |     |
| Sodium carboxymethylcellulose, 50 centipoise |       |       |       |       |       |       |      |       |       |       |      |     |
| Methylcellulose, 4,000 centipoise            | 2.0   | 2.0   | 2.0   | 4.0   | 4.0   | 4.0   |      |       |       |       |      | 2.0 |
| Glycerol                                     | 0.66  | 0.66  | 0.66  | 3.0   | 3.0   | 3.0   | 3.0  | 3.0   | 3.0   | 3.0   | 3.0  | 3.0 |
| Urea                                         | 0.5   | 0.5   | 0.5   | 1.0   | 1.0   | 1.0   | 1.0  | 1.0   | 1.0   | 1.0   | 1.0  | 1.0 |
| Diisobutylphenoxypolyethoxy ethanol          |       |       |       |       |       |       |      |       |       |       |      | 0.5 |
| Nonylphenoxypolyethoxy ethanol               |       |       |       |       |       |       |      |       |       |       |      |     |
| Sodium alkaryl polyether sulfate             |       |       |       |       |       |       |      |       |       |       |      |     |
| Alkylated aryl polyether alcohols            |       |       |       |       |       |       |      |       |       |       |      |     |
| Water                                        | 2.0   | 2.0   | 2.0   | 4.0   | 4.0   | 4.0   |      |       |       |       |      |     |
| Glycerol:vehicle                             | 100   | 100   | 100   | 100   | 100   | 100   | 100  | 100   | 100   | 100   | 100  | 100 |
| Urea:vehicle                                 | 1:3   | 1:3   | 1:3   | 1:1.3 | 1:1.3 | 1:1.3 | 1:3  | 1:3   | 1:3   | 1:3   | 1:3  | 1:2 |
| Spermicide:vehicle                           | 1:4   | 1:4   | 1:4   | 1:4   | 1:4   | 1:4   | 1:4  | 1:3   | 1:3   | 1:3   | 1:3  | 1:4 |
| Thickness of dried film in mils              | 2.0   | 2.0   | 2.0   | 4.0   | 4.0   | 4.0   | 4.0  | 4.0   | 2.0   | 2.0   | 2.0  | 2.0 |
| Thickness of foam in mils                    |       |       |       |       |       |       |      |       | 240   | 240   | 240  | 240 |

amples are given. These examples set forth specific solutions from which the articles of the present invention may be produced by evaporation of water in accordance with the procedures described above. In each instance, the composition includes sodium carboxymethylcellulose or methylcellulose as a vehicle, together with urea and other ingredients. The quantities given are by weight and are based upon the grams used with 100 grams of water.

The above compositions were tested for spermicidal effectiveness, the method followed being that described in "A Method of Testing the Relative Spermicidal Effectiveness of Contraceptives, and Its Application to Ten Commercial Products," Human Fertility, 5(4)-97, 1940, by R. L. Brown and C. J. Gamble.

In all instances the materials were instantly spermicidal at dilutions of 20 times (S/20).

Where the sheet-like material is in the form of a foam the area of the film-sheet, in square inches, should be at least 500 and preferably 1000 times or more the thickness of the film, while with a vigorously beaten foam, the area may be as small as or smaller than ten times the thickness of the material. Where a low concentration of spermicide occurs in the vehicle, this ratio will generally be larger than with higher concentrations, but with an unfoamed film 0.005 inch thick that contains about 14% of the spermicide, the area for a single use would be of the order of 9 to 16 square inches. With a film which had a concentration of 14% of spermicide and a thickness of 0.240 inch, about 2.5 square inches of the material should be used.

The spermicidal film or foamed material of the present invention lends itself readily to easy, inexpensive packaging, and a sufficient amount for a single use may be enclosed and hermetically sealed in an envelope of thermoplastic sheet material, such as polyethylene envelopes, in which case the material need not be completely dried, thereby partially eliminating the need for any humectant, and at the same time increasing the rapidity with which the dissolution of the material may start after application.

The invention in its broader aspects is not limited to the specific steps, processes and compositions shown and described but departures may be made therefrom within the scope of the accompanying claims without departing from the principles of the invention and without sacrificing its chief advantages.

This application is a continuation-in-part of Serial No. 597,861, filed July 16, 1956, and 690,452, filed October 16, 1957, both now abandoned.

What is claimed is:

- 5 1. A spermicidal sheet-like material comprising a sheet of non-deleterious, water soluble sodium carboxymethylcellulose, at least 5 milligrams of nonylphenoxypolyethoxyethanol, from about 20% to about 25% by weight of urea based on vehicle solids and from about 25% to about 45% by weight of glycerol.
- 10 2. A spermicidal material as claimed in claim 1 in which the area of the sheet is at least 10 times as great as its thickness.
- 15 3. A spermicidal material as claimed in claim 1 in which the sheet material is a foamed material.
- 20 4. A spermicidal material as claimed in claim 1 in which the sheet is from 0.001 to 0.0075 inch thick.
- 25 5. A spermicidal material as claimed in claim 1 in which the sheet is from 0.005 to 0.240 inch thick and is formed from a foam.
- 30 6. A spermicidal sheet-like material comprising a sheet of non-deleterious water soluble, carboxymethylcellulose, containing from 20% to 25% by weight of urea and from 1% to 50% by weight based on the carboxymethylcellulose of a spermicide selected from the group consisting of alkylated aryl polyether alcohols and a sodium alkylaryl polyether surfates and also containing about 25% to 40% by weight based on the carboxymethylcellulose of a humectant.
- 35 7. A spermicidal sheet-like material as claimed in claim 6 in which the humectant is glycerol.

#### References Cited in the file of this patent

##### UNITED STATES PATENTS

|    |           |                 |               |
|----|-----------|-----------------|---------------|
| 35 | 2,484,637 | Mattocks et al. | Oct. 11, 1949 |
|    | 2,563,593 | Engel           | Aug. 7, 1951  |
|    | 2,602,042 | Abbott          | July 1, 1952  |
|    | 2,693,438 | Ward            | Nov. 2, 1954  |

##### FOREIGN PATENTS

|    |         |           |               |
|----|---------|-----------|---------------|
| 40 | 150,013 | Australia | Feb. 12, 1953 |
|----|---------|-----------|---------------|

##### OTHER REFERENCES

45 Diserens: The Chemical Technology of Dyeing and Printing, Reinhold Publ. Co., New York (1948), p. 8.